

May 24, 1932.

D. M. SHANAFELT ET AL

1,859,803

APPARATUS FOR CONTINUOUS TREATMENT OF SHEET STEEL

Filed Aug. 3, 1929

4 Sheets-Sheet 1



May 24, 1932.

D. M. SHANAFELT ET AL

1,859,803

APPARATUS FOR CONTINUOUS TREATMENT OF SHEET STEEL

Filed Aug. 3, 1929

4 Sheets-Sheet 2



Fig. 5



Fig. 6

INVENTORS

Donald M. Shanafelt,  
George B. Nesbét,  
Albert F. Shonkwiler,  
By Justice Macklin ATTORNEY

May 24, 1932.

D. M. SHANAFELT ET AL

1,859,803

APPARATUS FOR CONTINUOUS TREATMENT OF SHEET STEEL

Filed Aug. 3, 1929

4 Sheets-Sheet 3



Fig. 7



Fig. 8.

INVENTORS

Donald M. Shanafelt,

George B. Nesbet,

Albert H. Shonkwiler,

BY Justice MacKlin ATTORNEY

May 24, 1932.

D. M. SHANAFELT ET AL

1,859,803

APPARATUS FOR CONTINUOUS TREATMENT OF SHEET STEEL

Filed Aug. 3, 1929

4 Sheets-Sheet 4



Fig. 9



Fig. 10



Fig. 11

INVENTORS  
Donald M. Shanafelt,  
George B. Nisbet,  
Albert H. Shonkwiler  
By Justice W. Macklin ATTORNEY

## UNITED STATES PATENT OFFICE

DONALD M. SHANAFELT, OF LAKEWOOD, GEORGE B. NISBET, OF CLEVELAND, AND ALBERT H. SHONKWILER, OF LAKEWOOD, OHIO, ASSIGNORS TO THE OTIS STEEL COMPANY, OF CLEVELAND, OHIO, A CORPORATION OF OHIO

## APPARATUS FOR CONTINUOUS TREATMENT OF SHEET STEEL

Application filed August 3, 1929. Serial No. 383,318.

This invention relates to heat treatment and finishing of steel sheets and the like, and more particularly to an apparatus for producing commercial sheets of the required degree of hardness and ductility at a very reduced cost.

Heretofore in the production of commercial sheets the practice has been to pass the sheets through a furnace in which the steel is heated to a temperature above the critical range, then slowly cooled to a temperature somewhat below the scaling temperature, and then placed in stacks and cooled in the open air to air temperature.

15 The next step has been to pass the sheets through a pickling bath, cold roll them, and then again place them in stacks in a box annealing furnace. In this last furnace the final heat treatment was given by very slowly heating and slowly cooling a large stack of material in a single mass. Such a process has proven very expensive, not only due to the numerous times the sheets must be handled, but also due to the great amount of time consumed. Furthermore, numerous handlings of the sheets between the various steps damaged and scratched the surfaces of a large number so that an additional rolling and extra pickling is often necessary.

20 Again, due to the size of the mass treated in the box annealing furnace, great heat is required to penetrate the inner sheets in a reasonable time, and quite generally the outer edge of all the sheets tend to heat too quickly while the inner portions of such a stack are not heated sufficiently. Uniformity of the finished sheets could be obtained only by a process so slow that instead of taking the required time, it was considered better practice to heat more quickly, even at the sacrifice of several sheets in each stack.

In the pickling process much of the corrosive action of the bath is utilized in removing scale or rust and mechanical irregularities resulting from handling of the sheets. Furthermore, after the sheets are pickled sufficiently, they must be washed to prevent further corrosive action of the bath. If exposed to the air when wet, there is a tendency for them to rust, losing much of the benefit of

the pickling. The same is true if they are left to the open air for an appreciable length of time. Again, exposure to the atmosphere allowed other foreign matter to drop on the sheets so that if rolled or subjected to heat without being treated, this foreign matter tended to imbed in or fuse onto the sheets or otherwise mar the surface.

It is one of the objects of our invention to reduce the expense of present methods, yet to produce commercial sheets of the required surface finish, and other characteristics, in a very much shorter time.

Another object is to produce sheets of such smooth finish which are very uniform in grain structure. By our process precisely the desired grain structure may be accurately controlled and the required drawability freedom from splits, cracks, laminations and the like is obtained, and the product may have a smooth surface finish, meeting the most exacting commercial requirements.

In the drawings—

Fig. 1 is a diagrammatic longitudinal section of a furnace adapted for carrying out our process;

Fig. 2 is a graph curve illustrating the temperatures of the various portions of the furnace in Fig. 1, as indicated in vertical alignment with Fig. 1;

Fig. 3 and 4 are respective continuations of the furnace and the graph shown in Figs. 1 and 2 respectively;

Fig. 5 and 6 are enlarged illustrations in the nature of a longitudinal section of such a furnace embodying means for continuous normalizing, pickling, rolling and annealing;

Fig. 7 is an enlarged section through the apparatus shown in Figs. 5 and 6 taken along the line 7—7;

Fig. 8 is an enlarged section through a portion of the apparatus taken on a plane indicated by the line 8—8 of Fig. 6;

Fig. 9 is a section through the portion of the furnace shown in Figs. 1 and 5, as indicated by the line 9—9.

Fig. 10 is a section through a portion of the furnace shown along line 10—10 of Fig. 6, and

Fig. 11 is a detail horizontal section taken as indicated by the line 11—11 of Figs. 5 and 9.

Referring more in detail to the drawings, our arrangement, as illustrated in Figs. 1 and 3, comprises a continuous furnace having a primary heating zone 1, a quick quenching zone 2, a secondary heating and tempering zone 3 and a slow cooling zone 4. The furnace is here shown as provided with the usual conveying rollers 5 mounted on water cooled shafts 6. The quick quenching zone is separated from the adjoining portions by means of flexible baffles such as chains 7, and is provided with cooling means, such for instance, as cool air or water pipes 8 in the upper portion.

This zone lowers the temperature of the sheets and yet allows the passage of gas through it from adjacent compartments. An open water tank 9 in this section through the quick quenching zone furnishes additional means for reducing the temperature therein.

It should be noted in this connection that the various zones intercommunicate. This is preferable to cause a non-oxidizing atmosphere to be retained in them, for the purpose of the prevention of scale or rust upon the sheets. Such an arrangement is particularly shown and described in our previous application, filed June 22, 1929, Serial No. 372,812.

An additional precaution in preventing the accumulation of scale and foreign matter on the sheets, due to such accumulation on the conveyors, may be taken by adding suitable scrapers, bearing against the rolls in the hottest zones, as indicated at 20 in Fig. 5.

The sheets enter the furnace, shown in Figs. 1 and 3, at the right, at air temperature or relatively cool, and pass into the compartment 1, wherein the temperature is raised to a degree above the critical range for the particular steel being treated, usually about 1750° to 1800° Fahrenheit. As discussed and illustrated in the above cited application, at such temperature the granular structure of the steel becomes very fine and regular. While in this condition the sheet passes through the quick quenching zone 2, wherein the temperature is suddenly reduced to a point below the critical temperature, for instance, a reduction of 200° or 300°. At this point the steel is relatively cool and the fine even grain structure just obtained is retained.

However, the sheet is quite hard, so the next step is to pass it into a reheating and tempering zone 3, in which the temperature of the sheet is increased fairly rapidly to an annealing temperature, for instance, to about 1200° F. It is then kept constantly at the desired temperature for a relatively long period of time, during which the grains "grow" or increase in size, yet retain their regularity and relative positions, so that the required

softness, ductility and drawability is obtained without in any way harmfully affecting the material.

Thereafter the sheet is passed into a long, much slower cooling compartment 4 and gradually cooled therein to a temperature at which it may be exposed to the open air, without further change, for instance, at a blue heat, or about 400° or 500°. Because of the exposure of the sheets over their entire area to the heat during this reheating and cooling, the annealing action is very uniform throughout and the time required to treat them is but a few minutes as compared to the large number of hours required in box annealing. Thus we may dispense with blue or box annealing and assure a controlled uniform treatment of each sheet.

The heating of the sheets may be very quick, as compared to raising the temperature of the large mass of stacked sheets as in box annealing alone.

The desired conditions may be exactly controlled. There are no difficulties from oxidation because the sheets are at all times enveloped in a neutral atmosphere of the products of combustion, which pass from the heating zones throughout the length of the furnace.

The proportions of the compartments shown by way of illustration are satisfactory for passing the sheets at a rate of one foot in about two seconds. Of course numerous variations may be made in the length of the various compartments if different speeds and combustion zone temperatures are used. As set forth in the application above cited, the use of the non-oxidizing atmosphere and scrapers will dispense with the use of rider sheets and permits more quickly heating and cooling the commercial sheets and also permits a more uniform heat in the upper and lower surfaces of each sheet. A sheet which has been carefully rolled before and well protected until placed in the furnace will be found to be in good condition for commercial use when the above operations have been performed.

These sheets however must necessarily be treated if they are for use in exposed positions requiring fine surface finishing, such as the exterior of automobile bodies, for example.

They are however perfectly satisfactory for such uses as concealed or rough finish surfaces, such as frame parts, oil pans, storage shelf, metal furniture and the like.

It will be seen however that the use of the process thus far described actually produces finished sheets which have all the desired characteristics for reasonably smooth surfaces, exact conditions of grain structure and drawability. Further treatment may be given them as by pickling and a cold rolling operation, which very slightly reduces the gauge and finishes the surface without noticeably altering the grain structure, lengthening the

sheet for example only from  $\frac{1}{2}$  to 1 inch in one hundred inches.

By a process using the annealing and normalizing apparatus and system, described in the above designated application, the sheets to be finished require the open annealing or normalizing in such a furnace, followed by pickling, and then either a dry cold rolling or, if the sheets require, a wet cold rolling. If the dry cold rolling is used, they may be immediately box annealed, which as stated, requires many hours, in fact several days, and again requires the finishing cold roll pass. If the sheets are wet cold rolled, that is, water used on the mill, they must again be pickled to remove the rust or results of oxidation occurring immediately, then box annealed and finish cold rolled as before.

It will be noted that the several days time required for cold rolling is eliminated by the method described, and also by the method employing additional steps which we will now describe, and by which the sheets are normalized, quenched, pickled, washed and cold rolled, and then annealed while controlling the grain growth, and thereafter slowly cooled and finally surface finished or "roller leveled". Thus we are enabled to produce, in one continuous operation, finished sheets for the most exacting requirements and all during a comparatively few minutes of time, eliminating all of the handling necessary to the present intermediate steps and the final box annealing or final roller levelling or separate cold roll pass.

The apparatus for carrying out all of these steps in one continuous process is best understood by reference to Fig. 5 and 6. As here shown, we employ a primary heating zone 11, quick cooling or quenching zone 12, re-heating zone 13, in the order named, said zones corresponding respectively to the zones 1, 2 and 3 of Fig. 1. These comprise the present normalizing system as described in the application above referred to. As stated, the sheets thus treated must be cleaned, pickled, cold rolled and again annealed, and all of this is accomplished by the subsequent continuous steps as follows:

Upon leaving the chamber 13, the sheets are subjected to a washing operation in which of course they are entirely cooled in the chamber 14, while passing over rollers, water being sprayed upon them from above and below through pipes 25 and 26, shown as connected with a common water supply pipe 30, as indicated in Fig. 7. A suitable baffle 27 defines one end wall of this chamber, the baffle being omitted in Fig. 7 for clearness.

A drainage opening, as indicated at 28 is provided to carry off the water from this chamber. The sets of conveying rollers in this chamber are arranged at different heights, forming an incline to permit drainage of the sheets. Further drainage is ef-

fected by maintaining the sheets sloping downwardly as they leave the washing chamber. The sheets then pass onto a chain or like conveyor 35 in the pickling chamber 15, shown as arranged to contain a suitable pickle bath through which the sheets are passed while carried on this conveyor. The length of this chamber is such as to permit the proper corrosive action of the pickling liquid, thoroughly cleaning the sheets. They are again passed along a downwardly and an upwardly sloping series of rollers in another washing chamber 16, also provided with spray pipes 25 and 26, and closed by a baffle wall 29. Here again surplus water may flow to a drainage opening as indicated.

In a subsequent chamber the rollers are shown positioned to move the sheets upwardly, allowing drainage, and are presented to one or more pairs (two being shown) of cold rollers 40. These very slightly reduce the thickness of the sheet without materially altering the grain structure, but producing almost exactly the desired finished gauge. The sheets pass from these cold rollers to the long annealing chamber 18, where heating burners 19 raise the temperature of the sheets to an annealing temperature, preferably of about 1200° F., and maintain this temperature, for a sufficient length of time to cause exactly the desired grain growth.

Passing beyond the zone of the burners, the sheets are allowed to very slowly cool still within the neutral atmosphere of the products of combustion to a temperature at which they are completely free from danger of scaling, due to exposure of the air, preferably somewhat below 400°, although 500 or 600° are satisfactory. This is substantially as described above and indicated by the graph curves on the charts Figs. 2 and 4. Here they are passed through the levelling or flattening rolls 50, which merely flatten and smooth the surfaces of the completely finished sheet. Subsequent cooling of the sheets is permitted in the open air, either singly or in stacks, as desired.

Due to the protection of the sheets throughout the length of the furnace and the freedom of the rollers from scale, due to the scrapers indicated at 20 on the rollers in the hot zones, the sheets are protected from foreign matter from above and below, and the intermediate treatment of washing, pickling, washing and subsequent rolling being while the sheets are still kept clean and free from foreign matter, the final resultant product is a very uniform sheet meeting the most exacting commercial requirements.

Reference may be had to an application, directed to construction and arrangement of said roller scrapers 20, filed by Messrs. Shonk-wiler and Macklin, Serial No. 372,812, filed June 22, 1929. By the use of these scrapers, rider sheets may be eliminated, and when

sheets are of the thinner gauges two or more sheets may be superimposed while passing through the furnace. The time for passing the sheets through the furnace being at a preferred speed of approximately one foot in two seconds, we may accomplish this complete treatment in the series of steps described in about thirty to forty minutes, depending on variations due to changes of conditions.

10 Thus in about one half an hour a sheet may be completely treated, whereas the time now required for the corresponding steps, particularly due to the box annealing, time 15 consumed in frequent handling, waiting for cooling between the steps, is actually quite a number of days.

We claim:

1. An apparatus for treating sheet steel 20 comprising a heat treating furnace, a pickling bath and a washing bath, and means for continuously passing the sheet steel through said furnace and baths in the order named, said furnace and baths being closed 25 to exclude outside atmosphere and communicating with each other, and means for heating said furnace and for maintaining therein and in said baths a non-oxidizing atmosphere.

30 2. An apparatus for treating sheet steel comprising a heat treating furnace, a pickling bath, a washing bath and levelling rolls arranged in succession in the order named, said baths and rolls being enclosed to exclude 35 outside atmosphere and said furnace being substantially sealed to exclude outside atmosphere, and said enclosures communicating with each other and with said furnace, and means for continuously progressing the 40 sheet steel through said furnace, baths and rolls in the order named, and means for heating said furnace and for maintaining a non-oxidizing atmosphere in said furnace and all of said enclosures.

45 3. An apparatus for treating sheet steel comprising two heat treating furnaces substantially sealed along their respective lengths to exclude outside atmosphere, and means for continuously progressing the sheet 50 steel along a given path extending through said furnaces, said furnaces being spaced apart from each other relative to the path of travel of the steel, a pickling bath and a 55 washing bath arranged along said path of travel in the order named and intermediate the furnaces, said baths being enclosed to exclude outside atmosphere, and said enclosures communicating with each other and with said furnaces and means for heating 60 said furnaces and for maintaining therein and in said enclosures a non-oxidizing atmosphere.

4. The combination with a furnace for 65 treating sheet steel and means for continuously progressing the steel therethrough and

along a given path, of a pickling bath and washing bath arranged in the order named along said path of travel, and means enclosing the baths sealed to exclude outside atmosphere therefrom, said means communicating with said furnace, and means for heating the furnace and maintaining therein and in said enclosing means a non-oxidizing atmosphere.

In testimony whereof, we hereunto affix 75 our signatures.

DONALD M. SHANAFELT.  
GEORGE B. NISBET.  
ALBERT H. SHONKWILER.

80

85

90

95

100

105

110

115

120

125

130